# EUROPEAN PATENT SPECIFICATION

(11) **EP 0 241 812 B1**
(45) Date of publication and mention of the grant of the patent: **08.09.1993**
(21) Application number: 87104872.4
(22) Date of filing: 02.04.1987
(51) Int. Cl.: C22C 37/04

(54) **Ferritic ductile cast iron for elevated temperature applications**
Ferritisches Kugelgraphit-Gusseisen für den Einsatz bei erhöhter Temperatur
Fonte ductile ferritique pour applications à température élevée

(30) Priority: 07.04.1986 US 848612
(43) Date of publication of application: 21.10.1987
(73) Proprietor: GENERAL ELECTRIC COMPANY, Schenectady New York 12305 (US)
(72) Inventor: Farrell, Thomas Raymond, Scotia, New York, 12302 (US)
(74) Representative: Pratt, Richard Wilson

(56) References cited:
- EP-A- 0 131 092
- DE-A- 1 758 038
- GB-A- 2 134 135
- GB-A- 2 147 007
- GIESSEREI-PRAXIS, Nr. 3,4, 1985, Berlin, D; K. ROEHRIG: "Eigenschaften von unlegiertem und niedriglegiertem Gusseisen mit Kugelgraphit bei erhöhten Temperaturen"

## Description

This invention relates generally to a ferritic ductile cast iron composition having improved elevated temperature properties, and particularly relates to a ferritic ductile cast iron composition which is substantially immune to elevated temperature brittleness.

Ferritic ductile cast iron is an important engineering alloy having several advantages over steel products, including low material cost and castability. However, for elevated temperature applications, steel products tend to be chosen for their superior mechanical properties. The phenomenon of elevated temperature brittleness (ETB) is in part responsible for the inability of ductile iron to compete with steels in such applications. This is particularly true in cases where good thermal fatigue resistance is required such as turbine casing applications, high pressure vessels and engine components.

Although the phenomenon of brittleness of ferritic ductile cast iron at elevated temperatures has been known for many years, little has been done to understand it. It has been shown that ETB manifests itself within a fairly narrow elevated temperature region by its pronounced effect on various physical properties. Such effects include reduced tensile strength, reduced tensile ductility and reduced low cycle fatigue resistance. The cause of these adverse effects on such material properties has been found to be the direct result of intergranular fracture.

It has also been determined that the temperature at which ductility is minimized is variable and is strain rate dependent. For the iron in question, this temperature occurs at 400 °C (725 °F) and 500 °C (932 °F) for strain rates of 2.8 x 10⁻⁴ sec ⁻¹ and 1.4 x 10⁻², respectively. However, even with this knowledge, a solution to the problem of ETB has heretofore eluded the foundry industry.

GB-A-2147007 discloses a spheroidal graphite ferrite cast iron having magnesium and sulfur contents ranging, respectively, from 0.02 to 0.15 % and from 0 to 0.03 % by weight which is said to have high resistance to oxidation at the blue brittleness temperature and a high degree of toughness and fracture resistance at high temperatures.

DE-A-1758038 discloses a ductile nodular graphite cast iron having magnesium and sulfur contents ranging, respectively, from 0 to 0.01 % and 0.02 to 0.07 % by weight. This cast iron has a microstructure containing less than 10 % by weight pearlite.

Accordingly, a need exists for a ferritic ductile cast iron which exhibits improved elevated temperature properties including improved tensile ductility, improved low cycle thermal fatigue capability and reduced intergranular fracture.

The present invention has been developped to overcome the temperature related drawbacks of conventional iron by providing a new ferritic ductile cast iron having improved strength, ductility and thermal fatigue resistance at elevated temperatures. Extensive testing of the effects of chemical composition, strain rate and temperature have led to the discovery that certain ductile iron compositions may be produced which are substantially immune to ETB and which exhibit improved fatigue properties comparable to several common steels.

The characteristics of ETB have been found to be similar to metal induced embrittlement in that both phenomena exhibit onset and recovery and a strain rate effect. Reduced mechanical properties associated with ETB have been found to be the direct result of the development of intergranular fracture which develops upon reaching maximum load.

The mechanism responsible for ETB appears to be magnesium assisted sulfur segregation. The identification of this mechanism is based upon correlations between magnesium, sulfur and the occurrence of ETB. As a result of this realization, ferritic ductile iron compositions containing low sulfur and/or low magnesium levels have been formulated in accordance with the invention so as to be substantially immune to ETB.

The occurrence of ETB is studied through examination of a value defined as a "ductility ratio" which is the elevated temperature ductility measured at 425°C (800°F) divided by the ductility at room temperature. The ductility ratio separates ETB effects from other effects on ductility. Alloying and microstructure effect both room temperature ductility as well as elevated temperature ductility so as to leave the ductility ratio unchanged. However, ETB affects only elevated temperature ductility and thus dramatically changes the ductility ratio. Reliance on elevated temperature ductility alone as an indicator of ETB would provide a much weaker correlation due to the clouding or obfuscating effects of alloying and microstructure.

Most of the presently marketed ferritic ductile cast irons are susceptible to ETB and would therefore offer limited temperature capability. By eliminating ETB as taught by the invention, an improved alloy is obtained which has comparable elevated temperature fatigue resistance to plain carbon of low alloy steels.

It is therefore a primary object of the invention to provide a ferritic ductile cast iron composition which is rendered substantially immune to ETB by controlling and limiting the residual concentrations of magnesium and sulfur.

According to the present invention there is provided a ferritic ductile cast iron composition characterized in that it comprises a residual quantity of sulfur in a weight percentage of no greater than 0.015 and in that the combination of residual quantities of magnesium and sulfur into the parameter (Mg + 4.5 S) in weight percentage is no greater than 0.070, and graphite, said graphite comprising 99 % by volume ASTM Type I and/or ASTM Type II graphite and 1 % by volume of ASTM Type IV graphite.

In a preferred embodiment the iron composition microstructure includes a quantity of pearlite of 3 % by weight.

In another preferred embodiment the iron composition of the present invention is a subcritically annealed iron composition, and more preferably an iron composition critically annealed at 900 °C and subcritically annealed at 720 °C.

In a still preferred embodiment the iron compositions of the present invention have a ductility ratio which is not inferior to 0.6.

Various other objects, features and attendant advantages of the present invention will be more fully appreciated as the same becomes better understood from the following detailed description when considered in connection with the accompanying tables and drawings wherein:
Table 1 is a listing of various ferritic ductile cast iron heat chemistries identifying each component in weight percent;
Table 2 is a listing of ferritic ductile cast iron heat treatments and microstructures;
Table 3 is a listing of fracture characteristics of heats G and H;

Figure 1 is a fitted plotting of tensile area reduction of heats B, E, G and H as a function of temperature;
Figure 2 is a fitted plotting of the fracture strength of heats B, E, G and H as a function of temperature;
Figure 3 is a metallographic fracture sectioning of a tensile specimen taken from heat G identifying areas of intergranular fracture and shrinkage porosity (enlarged 200X) tested at 425°C (800°F), nital etch;
Figure 4 is a metallographic fracture sectioning of a tensile specimen taken from heat H (enlarged 200X) tested at 425°C (800°F), nital etch;
Figure 5 is a fitted plotting of a dependence of elevated temperature ductility of ferritic ductile cast iron on magnesium and sulfur content wherein an ETB immunity region is defined between the plot axes and the line Mg + 4.5S = 0.07;
Figure 6 is a fitted plotting of tensile area reduction as a function of strain rate and temperature of heats G and H;
Figure 7 depicts fracture stress as a function of strain rate and temperature for heats G and H.
Figure 8a is a view of the fracture surface of a tensile specimen of heat G identifying areas of intergranular fracture and shrinkage porosity (enlarged 200X) tested at 370°C (700°F), at a strain rate of 4.4 x 10⁻⁵ sec ⁻¹;
Figure 8b is a view of the fracture surface of a tensile specimen of heat G identifying areas of intergranular fracture and shrinkage porosity (enlarged 1000X), tested at 370°C (700°F), at a strain rate of 4.4 x 10⁻⁵ sec ⁻¹;
Figure 9a is a view of the fracture surface of a tensile specimen of heat H (enlarged 200X), tested at 370°C (700°F), at a strain rate of 4.4 x 10⁻⁵ sec ⁻¹;
Figure 9b is a view of the fracture surface of a tensile specimen of heat H (enlarged 1000X), tested at 370°C (700°F), at a strain rate of 4.4 x 10⁻⁵ sec ⁻¹;
Figure 10 is a transmission electron microscope relief replica fractograph of the intergranular fracture area on a specimen of heat G (enlarged 10,000X);
Figure 11 is a transmission electron microscope relief replica fractograph of the shrinkage area on a specimen of heat G (enlarged 10,000X);
Figure 12 depicts the intergranular fracture area on a specimen of heat E identifying areas of intergranular fracture and shrinkage porosity (enlarged 500X), prestrained at 425°C (800°F);
Figure 13 shows the low cycle fatigue behavior of ferritic ductile cast iron tested at 425°C (800°F);
Figure 14a depicts a fracture surface of a specimen of heat B (enlarged 75X), low cycle fatigue tested at 425°C (800°F);
Figure 14b depicts a fracture surface of a specimen of heat B (enlarged 500X), low cycle fatigue tested at 425°C (800°F);
Figure 15a depicts the fracture surface of a specimen of heat H (enlarged 75X), low cycle fatigue tested at 425°C (800°F);
Figure 15b depicts the fracture surface of a specimen of heat H (enlarged 500X), low cycle fatigue tested at 425°C (800°F);
Figure 16 shows the effect of strain rate on elevated temperature ductility of ferritic ductile cast iron; and
Figure 17 is a comparison of low cycle fatigue properties of heats H, I, J and K to cast steel A216WCC and plate steel A516-Gr55 (transverse orientation) at 425°C (800F).

In order to better understand the phenomenon of elevated temperature brittleness in ferritic ductile cast iron, an in-depth investigation was conducted to study the effects of chemical composition, strain rate and temperature on ETB. Twenty-six different material compositions representing a wide range of ferritic ductile cast iron chemistry were selected for study. The chemical composition of each heat is set forth in Table 1 and a description of each heat in terms of heat treatment and microstructure is set forth in Table 2.

The general mechanical behavior of ferritic ductile cast iron in the ETB regime was studied with the aid of tensile and low cycle fatigue testing. The tensile tests were in four series, the first series involving air testing 6.35 mm diameter test specimens from room temperature to 650°C (1200°F) using standard ASTM practice. Primary emphasis was on heats B, E, G and H. The strain rate in these tests was 8.3 x 10⁻⁵ sec ⁻¹, up to yielding and then 8.3 x 10⁻⁴ sec ⁻¹ to fracture.

Microscopic examination of failed tensile and fatigue test specimens was performed using longitudinal sectioning, scanning electron microscopy, relief replica transmission electron microscopy and energy dispersive X-ray analysis.

Figure 1 shows the reduction in area from the first series of tensile tests as a function of temperature for heats B, E, G and H. The ETB regime is sharply delineated at 425°C (800°F). It is important to note that heat H appears substantially unaffected by ETB and clearly shows less brittleness than the other heats.

The ETB regime is less clearly seen in the fracture stress data plotted in Figure 2. Even so, heat H, a preferred heat, displays a higher fracture stress although all heats show a rapid decline in fracture stress with increasing temperature. Metallographic sectioning of 425°C (800°F) tested specimens of heats G and H indicate the presence of intergranular fracture in heat G, as shown in Figure 3, while none was found in heat H, as shown in Figure 4.

From the room temperature and 425°C (800°F) tensile testing of the entire group of heats listed in Table 1, the ratio of ETB minimum area reduction to room temperature area reduction, expressed as a ductility ratio "DR" is seen to correlate with the combination of magnesium (Mg) and sulfur (S) content of each heat. This correlation is shown in Figure 5. The DR value clearly separates ETB effects from variations in mechanical properties due to alloying or microstructure. A ductility ratio of near unity implies behavior to heat H while a ratio near one-fourth implies behavior similar to heat G. Clearly, a poor ductility ratio is associable with elevated Mg and S content. By maintaining the parameter (Mg + 4.5S) below 0.07, ETB is avoided. This represents a triangular region as shown in the left side of Figure 5. The fact that ETB behavior is well defined by the residual Mg and S content strongly suggests a major role of these two elements.

Figure 5 includes data from heats containing degenerate graphite (ASTM Type IV). Such structures usually reflect Mg "fade" or an insufficient Mg addition, and may be unacceptable in spite of their immunity to ETB.

The second series of constant displacement tensile tests were performed on a Gleeble 1500 test machine. Data from these tests provides evidence of the effect of strain rate on ETB. Figure 6 shows area reduction data for heats G and H. The relative superiority in ductility and lower temperature tinimum of heat H is again clear. Moreover, it is clear that the temperature of minimum area reduction is 130°C (235°F) higher for the higher strain rate. Additionally, the ETB temperature range (the range over which the area reduction is reduced) is greater for the higher strain rate. The effect of strain rate on fracture stress is shown in Figure 7.

The difference in embrittlement observed between heats G and H (among others) may be related, by fractography, to the degree of intergranular fracture as shown in Figures 8a and 8b. The pronounced embrittlement of heat G is associated with extensive intergranular fracture and the presence of shrinkage porosity within the intergranular fracture region. Figures 9a and 9b show the classical dimpled rupture behavior that dominates the less brittle heat H.

A quantitative description of the extent of intergranular fracture is given in Table 3 and noted in Figure 6 for many of the Gleeble machine tested specimens. A representative transmission electron microscope relief fractograph of an intergranular surface tensile tested at 425°C (800°F) is shown in Figure 10. Likewise, transmission electron microscope fractography confirms that porosity is the result of shrinkage during solidification, as shown in Figure 11.

A third series of two-stage interrupted tensile tests provides a clear delineation of intergranular fracture areas and reveals that such fracture initiates at shrinkage pores. These tests involved first preloading the test bar at 425°C (800°F) using standard ASTM tensile test procedures and then interrupting the test prior to reaching maximum load. The pre-loaded bars were then tested at room temperature to reveal fracture initiation behavior. Figure 12 shows a scanning electron microscope fractograph from one of these interrupted tensile tests. It is clear from these tests that fracture initiates at shrinkage pores in the ETB temperature range.

Strain controlled low cycle fatigue test results are presented in Figure 13. A clear difference in fatigue resistance is evident. Those heats exhibiting superior low cycle fatigue resistance also have reduced elevated temperature brittleness response. These results correlate with the Mg and S correlation (DR ratio) discussed above.

A scanning electron microscope fractographic examination of a heat B low cycle fatigue specimen identifies intergranular fracture and associated shrinkage porosity as shown in Figures 14a and 14b. Examination of heat H shows only transgranular fracture in Figures 15a and 15b.

The above test results provide evidence as to the ETB fracture mechanism. From the observation that intergranular fracture initiates from the shrinkage pores, the fracture mechanism can be related to the last liquid to solidify or to segregation. A dependence of such fracture upon Mg and S is also shown. Since Mg is relatively insoluble in iron, segregation to grain boundaries should occur in the last liquid to solidify. Mg is usually combined and, since it is added to the melt to scavenge impurities such as sulfur, some minor amount of magnesium sulfide (MgS) should be present in the melt during solidification. The amount of MgS residing in the grain boundaries would depend on many factors including melt chemistry, magnesium additions and time. The time factor would explain the benefit of magnesium "fade" which results in ASTM Type IV graphite and improved fatigue resistance. Despite these variables, the residual amounts of magnesium and sulfur are directly relatable to the occurrence or immunity to ETB.

Once formed, MgS is unstable at temperature above room temperature and, with time, decomposes into magnesium oxide (MgO) and free sulfur upon cooling from solidification or during heat treatment. In bulk form, sulfur has a boiling point of 455°C (855°F), which is coincidentally close to the temperatures observed for ETB. All of the above suggest that ETB is the result of magnesium assisted sulfur segregation with sulfur as the embrittler and magnesium as the transport mechanism. This appears to explain the interrelation or synergy between magnesium and sulfur in which lower sulfur levels allow for higher magnesium levels before observing ETB.

The strain rate effect can be seen more clearly in Figure 16 which shows a plot of the temperature of minimum area reduction versus strain rate for heat G. Onset and recovery temperatures can be identified from the temperatures at which heats G and H show comparable area reduction above and below the minimum. From Figure 16 a clearer understanding of the strain rate effect on ETB affected heats is obtained. This behavior has similarities to metal induced embrittlement.

The temperature for onset of ETB can be related to the mobility of sulfur, and as such should be diffusion controlled. That is, that in order for intergranular fracture to contribute significantly to the overall fracture process, sulfur must be mobile enough to keep pace with the damage rate. At low temperatures and/or high strain rates, sulfur is presumably not mobile enough to keep pace with the damage rate and only ductile fracture occurs because of insufficient time for the movement of sulfur.

Recovery may occur from the possibility that free sulfur oxidizes and is prevented from causing further embrittlement. This process would also be diffusion controlled and would be predominant at the specimen surface. That is to say that at higher temperatures and longer times (slow strain rates), oxygen may have sufficient mobility to reach intergranular crack fronts and prevent further crack advance.

Whatever the mechanism for ETB may be, the Mg-S correlation indicates that low sulfur is highly important. The reduction of sulfur levels leads to wider ranges of acceptable Mg levels and to a lower propensity for degenerated graphite.

It can be appreciated that the present invention is based on the identification of a number of heats of ferritic ductile iron which do not exhibit ETB. Of particular interest is heat H which is substantially immune to ETB. A comparison of the fatigue properties of some of these heats with two commonly used steels is shown in Figure 17. The ductile iron heats are comparable in fatigue capability to these steels.

Based on the test results discussed above, the following observations can be made regarding the elevated temperature brittleness of ferritic ductile iron:
1) Elevated temperature brittleness acts to reduce tensile strength, tensile ductility and fatigue resistance.
2) ETB is observed in an elevated temperature range which is strain rate dependent. For a strain rate of 4.4 x 10⁻⁵ sec ⁻¹, the temperature range is 310°C (590°F) to 490°C (914°F), while for a strain rate of 2.0 x 10⁻² sec ⁻¹, the range is 370°C (700°F) to 760°C (1400°F).
3) The temperature at which tensile area reduction is minimum moves to higher temperatures with increasing strain rate. For a strain rate of 4.4 x 10⁻⁵ sec ⁻¹, the area reduction minimum occurs at 400°C (725°F), while for a strain rate of 2.0 x 10⁻² sec ⁻¹, the minimum occurs at 530°C (986°F).
4) Onset and recovery occurs similar to metal induced embrittlement.
5) Intergranular fracture is associated with reduced tensile ductility and at the ductility minimum can account for up to 35 percent of the fracture surface.
6) Intergranular fracture initiates at shrinkage pores.
7) The ductility ratio, which is the ratio of area reduction at the ductility minimum temperature (taken as area reduction at 425°C (800°F RA) to that at room temperature, correlates with magnesium and sulfur levels. Low magnesium and/or low sulfur levels lead to relative immunity to ETB. A value of DR near one-fourth indicates full ETB while a value near unity indicates relative immunity to ETB.
8) ETB appears to be the result of magnesium assisted sulfur segregation. The residual percent by weight level of sulfur and magnesium combined into the parameter (Mg + 4.5S) should be maintained below 0.070 percent by weight in order to avoid ETB.
9) Low cycle fatigue life is severely affected by ETB in a similar manner as tensile ductility.

**Table 1**

| Ferritic Ductile Cast Iron Heat Chemistries (Wt. Pct.) | | | | | | | | | | | | | |
|---|---|---|---|---|---|---|---|---|---|---|---|---|---|
| Heat | C | Si | Ni | Mo | Mn | P | Mg | S | Ti | V | Al | Cu | Cr |
| A | 3.60 | 2.29 | 0.89 | 0.05 | 0.22 | .015 | .052 | .009 | .011 | | .020 | .045 | .089 |
| B | 3.60 | 2.20 | 0.38 | 0.74 | 0.23 | .018 | .048 | .016 | .015 | | .039 | .035 | .063 |
| C | 3.38 | 3.07 | 0.26 | 0.47 | 0.10 | .020 | .057 | .007 | | | | | |
| D | 3.69 | 2.37 | 0.05 | 0.61 | 0.22 | .017 | .061 | .018 | .025 | .008 | .056 | .031 | .063 |
| E | 3.70 | 2.78 | 0.15 | 0.67 | 0.19 | .016 | .048 | .016 | .029 | | .052 | .051 | 0.64 |
| F | 3.50 | 2.38 | 0.75 | 0.50 | 0.10 | .016 | .038 | .008 | .024 | .024 | .039 | .044 | .083 |
| G | 3.43 | 2.21 | 1.23 | 0.40 | 0.09 | .017 | .053 | .009 | .024 | .024 | .029 | .048 | .075 |
| H | 3.55 | 2.63 | 0.13 | 0.61 | 0.09 | .017 | .023 | .008 | .025 | .022 | .059 | .045 | .071 |
| I | 3.61 | 2.72 | 0.07 | 0.59 | 0.07 | .019 | .029 | .005 | .020 | .030 | | .010 | .030 |
| J | 3.46 | 3.00 | 0.73 | 0.80 | 0.09 | .022 | .025 | .008 | .033 | .033 | .115 | .019 | .061 |
| K | 3.55 | 3.29 | 0.59 | 0.95 | 0.07 | .020 | .026 | .005 | .021 | .040 | | .010 | .050 |
| L | 3.43 | 3.06 | 0.60 | 1.35 | 0.07 | .024 | .017 | .005 | | | | | |
| M | 3.55 | 2.60 | 0.96 | | 0.17 | .007 | .033 | .007 | | | .007 | .022 | .080 |
| N | 3.35 | 2.53 | 0.13 | 0.03 | 0.05 | .020 | .036 | .009 | .014 | .026 | .034 | .043 | .055 |
| O | 3.54 | 2.86 | 0.88 | 0.57 | 0.02 | .018 | .025 | .009 | | | .031 | | .056 |
| P | 3.38 | 2.70 | 1.51 | 0.66 | 0.02 | .014 | .035 | .005 | .025 | .041 | .020 | .026 | .051 |
| Q | 3.45 | 2.72 | 0.55 | 0.68 | 0.05 | .018 | .022 | .008 | .024 | .040 | | .010 | .090 |
| R | 3.60 | 3.30 | 0.49 | 0.01 | 0.02 | .005 | .022 | .007 | .027 | .010 | | .010 | .010 |
| T | 3.60 | 2.71 | 0.48 | 0.01 | 0.02 | .008 | .029 | .009 | .034 | .010 | | .010 | .120 |
| V | 3.56 | 2.60 | 0.03 | 0.00 | 0.24 | .024 | .050 | .004 | .004 | .002 | .015 | | .028 |
| W | 3.66 | 2.52 | 0.03 | 0.00 | 0.24 | .022 | .052 | .004 | .008 | .007 | .018 | | .027 |
| X | 3.66 | 2.50 | 0.04 | 0.01 | 0.25 | .028 | .061 | .003 | .016 | .011 | .020 | | .036 |
| Y | 3.64 | 2.16 | | | 0.28 | .020 | .016 | .006 | | | | | |
| Z | 3.49 | 2.68 | | | 0.38 | .020 | .018 | .008 | | | | | |

**Table 2**

| Ferritic Ductile cast Iron Heat Microstructure | | | |
|---|---|---|---|
| Heat | Heat(1) Treatment | ASTM Graphite % Type I & II / % Type IV | % Pearlite |
| A | FA | 99/1 | 5 |
| B | FA | 99/1 | 7 |
| C | FA | 99/1 | 7 |
| D | FA | 99/1 | 5 |
| E | FA | 99/1 | 5 |
| F | SCA | 99/1 | 10 |
| G | SCA | 99/1 | 7 |
| H | SCA | 99/1 | 3 |
| I | FA | 99/1 | 3 |
| J | SR | 99/1 | 5 |
| K | SCA | 99/1 | 5 |
| L | SCA | 30/70 | 5 |
| M | SCA | 99/1 | 5 |
| N | SCA | 99/1 | 3 |
| O | FA | 10/90 | 7 |
| P | FA | 99/1 | 5 |
| Q | SCA | 50/50 | 3 |
| R | SCA | 99/1 | 3 |
| T | SCA | 99/1 | 5 |
| V | SR | 99/1 | 3 |
| W | SR | 99/1 | 7 |
| X | SR | 99/1 | 3 |
| Y | SCA | 20/80 | 3 |
| Z | SCA | 10/90 | 3 |

| | | | |
|---|---|---|---|
| (1) SR - As-cast with 595°C stress-relief anneal SCA - Sub-critical anneal only (720°C) FA - Full anneal (critical anneal at 900°C and sub-critical anneal at 720°C) | | | |

**TABLE 3**

| FRACTURE CHARACTERISTICS OF HEATS G AND H | | | | | | |
|---|---|---|---|---|---|---|
| HEAT | SPEC NO. | STRAIN RATE -1 SEC. | TEMP (°C) | TEMP (°F) | % INTERG. FRAC. | % SHRINK POROS. |
| G | 8 | 4.4 X 10⁻⁵ | 370 | 700 | 22.7 | 3.0 |
| | 3 | " | 425 | 800 | 36.5 | 3.8 |
| | 13 | 2.0 x 10⁻² | 425 | 800 | 0.0 | 5.9 |
| | 17 | " | 480 | 900 | 15.9 | 3.5 |
| | 10 | " | 540 | 1000 | 35.4 | 6.2 |
| | 15 | " | 595 | 1100 | 17.6 | 5.1 |
| H | 5 | 4.4 X 10⁻⁵ | 425 | 800 | <1.0 | 2.3 |
| | 10 | 2.0 X 10⁻⁵ | 540 | 900 | <1.0 | 1.1 |

## Claims

1. A ferritic ductile cast iron composition characterized in that said composition comprises a residual quantity of sulfur in a weight percentage of no greater than 0.015 and in that the combination of residual quantities of magnesium and sulfur into the parameter (Mg + 4.5S) in weight percentage is no greater than 0.070, and graphite, said graphite comprising 99% by volume ASTM Type I and/or ASTM Type II graphite and 1 % by volume of ASTM Type IV graphite.

2. The iron composition of claim 1, characterized in that it further comprises a microstructure including a quantity of pearlite of 3% by weight.

3. The iron composition of claim 1 or 2, wherein said iron composition is a sub-critically annealed iron composition.

4. The iron composition of claim 1 or 2, characterized in that said iron composition is critically annealed at a temperature of 900°C and sub-critically annealed at 720°C.

5. The iron composition according to any one of claims 1 to 4 characterized in that it has a electricity ratio (DR), defined as the elevated temperature ductility measured at 425°C (800°F) divided by the ductility at room temperature, which is not inferior to 0.6.

## Patentansprüche

1. Eine ferritische duktile gegossene Eisenzusammensetzung, dadurch gekennzeichnet, daß die genannte Zusammensetzung eine Restmenge Schwefel von nicht mehr als 0,015 Gew.-% und daß die Kombination der Restmengen von Magnesium und Schwefel in dem Parameter (Mg+4,5S) nicht größer als 0,070 Gew.-% ist und Graphit umfaßt, wobei der Graphit 99 Volumen-% vom ASTM Typ I und/oder vom ASTM Typ II und 1 Volumen-% vom ASTM Typ IV umfaßt.

2. Die Eisenzusammensetzung nach Anspruch 1, dadurch gekennzeichnet, daß sie weiter ein Gefüge aufweist, das eine Menge von 3 Gew.-% Perlit einschließt.

3. Die Eisenzusammensetzung nach Anspruch 1 oder 2, worin die genannte Eisenzusammensetzung eine unterkritisch geglühte Eisenzusammensetzung ist.

4. Die Eisenzusammensetzung nach Anspruch 1 oder 2, dadurch gekennzeichnet, daß die genannte Eisenzusammensetzung bei einer Temperatur von 900°C kritisch geglüht und bei einer Temperatur von 720°C unterkritisch geglüht ist.

5. Die Eisenzusammensetzung nach einem der Ansprüche 1 bis 4, dadurch gekennzeichnet, daß sie ein Duktilitätsverhältnis (DV), definiert als die Duktilität bei erhöhter Temperatur, gemessen bei 425°C (800°F), dividiert durch die Duktilität bei Raumtemperatur, aufweist, das nicht kleiner als 0,6 ist.

## Revendications

1. Composition de fonte ductile ferritique caractérisée en ce que ladite composition comprend une quantité résiduelle de soufre en un pourcentage en poids qui n'est pas supérieur à 0, 015 et en ce que la combinaison de quantités résiduelles de magnésium et de soufre dans le paramètre (Mg+4,5S) en pourcentage en poids n'est pas supérieure à 0,070, et du graphite, ledit graphite comprenant 99% en volume de graphite de type I ASTM et/ou de type II ASTM et 1% en volume de graphite du type IV ASTM.

2. Composition de fonte selon la revendication 1, caractérisée en ce qu'elle comprend, en outre, une microstructure comprenant une quantité de perlite de 3% en poids.

3. Composition de fonte selon la revendication 1 ou 2, dans laquelle la composition de fonte est une composition de fonte recuite en dessous du point critique.

4. Composition de fonte selon la revendication 1 ou 2, caractérisée en ce que ladite composition de fonte est recuite au-dessus du point critique, à une température de 900°C et est recuite de façon sous-critique à une température de 720°C.

5. Composition de fonte selon l'une quelconque des revendications 1 à 4, caractérisée en ce qu'elle présente un rapport de ductilité (DR), défini comme étant le quotient de la ductilité à température élevée, mesurée à 425°C (800°F), par la ductilité à la température ambiante, qui n'est pas inférieur à 0,6.
